

Dec. 24, 1968

W. A. FAHLBUSCH  
COLORING ANODIZED ALUMINUM

3,418,219

Filed March 29, 1966



INVENTOR.  
WILLIAM A. FAHLBUSCH

BY

*Francis J. Mallega*

ATTORNEY

3,418,219

## COLORING ANODIZED ALUMINUM

William A. Fahlbusch, Arlington Heights, Ill., assignor to  
Martin-Marietta Corporation, New York, N.Y., a corporation of Maryland

Filed Mar. 29, 1966, Ser. No. 538,389

12 Claims. (Cl. 204—38)

The present invention is related to the coloring of anodized aluminum and, more particularly, to the production of a black color on anodized aluminum.

In the past there have been proposed a number of processes for producing colored anodized metal, especially black colored aluminum. These processes are generally of two kinds. First a color may be introduced into the pores of an anodic film on the surface of anodized aluminum by the use of one or more colored dyes carried in either an aqueous bath or an organic vehicle. The second type of process involves the formation of a colored precipitate in the pores of the anodic film. Such a colored precipitate is often a metallic sulfide and, more particularly, is produced by a metathetical reaction wherein a metal ion is absorbed into the anodic pores followed by the subsequent absorption of sulfide ion therein.

The aforementioned prior art processes have certain disadvantages. With very few exceptions, organic colorations are subject to fading through the action of light, oxidation and the like. With respect to the prior art metallic sulfide colors, it is very difficult to obtain uniform coloration in any reasonable length of time. Since the depth of color is dependent upon the relative completeness of diffusion, time, often amounting to up to about one hour, must be allowed to permit diffusion to occur. The fact that a solid product, i.e., the sulfide precipitate, is forming in narrow pores in the anodized layer during diffusion slows down the rate at which the color develops. In view thereof it is difficult to achieve a uniform, deeply colored aluminum by the usual metathetical reactions proposed heretofore. As far as is known, the art has not been provided with a commercially acceptable process whereby the disadvantages enumerated hereinbefore can be overcome.

It has now been discovered that by means of a novel combination of ingredients employed in a novel manner deep, commercially satisfactory, black colorations can be produced in anodized metal.

It is an object of the present invention to provide a novel process for the production of black-colored anodized metal.

Another object of the present invention is to provide a novel composition of matter useful in the formation of black-colored anodized aluminum.

A further object of the present invention is the provision of novel coloring solutions for use in the coloration of anodized aluminum.

Other objects and advantages will become apparent from the following description taken in conjunction with the drawing in which the figure shows a schematic outline of an anodizing and coloring process involving use of the present invention.

Generally speaking, the present invention contemplates a coloring process wherein a porous anodized surface is impregnated with an aqueous solution containing in solution a substance capable of donating a precipitant ion (e.g., sulfide ion) at temperatures in excess of about 200° F. and stable in aqueous solution at temperatures below about 100° F. and an ion capable of reacting with the precipitant ion to form a colored precipitate which is insoluble in water and heating the thus impregnated anodized surface to a temperature in excess of about 250° F. for at least about one or two minutes whereby the anodized surface is colored. Heating times can be up to any

practical length of time and are principally dependent upon temperature. Longer times are employed at lower temperatures and shorter times are employed with higher temperatures.

5 The present invention further contemplates as a composition of matter a coloring impregnant for coloring anodized metal comprising an aqueous solution containing in solution metalliferous ion capable of reacting with the sulfide ion to form a colored sulfide which is insoluble in water, at least an amount of a substance capable of donating sulfide ion at temperatures in excess of about 200° F. and stable in aqueous solution at temperatures below about 100° F. effective to provide sufficient sulfide ion under reaction conditions to react with said metalliferous ion, a thickening agent in an amount effective to induce in the aqueous solution a workable viscosity for the means by which the coloring impregnant is applied to the anodized metal and a stabilizing agent. In addition, the aqueous solution can contain dispersed therein an insoluble substance designated in this specification and claims as a flattening agent.

10 The ion capable of reacting with the precipitant sulfide ion used in the coloring process of the present invention is at least one member of the group consisting of the ions of cobalt, copper, antimony, nickel, molybdenum, iron, and bismuth. In order to obtain a stable black coloration in the anodized surface, it is advantageous to employ ions of cobalt, nickel or iron. It is pertinent to note that the ion employed in solution can be not only a simple hydrated ion of a metal mentioned hereinbefore but also a complex ion which contains as a part thereof a metal mentioned hereinbefore. When a complex ion is employed, it is necessary that the complex ion be capable of thermal degradation at a temperature below about the heating temperature. The use of the term "precipitant ion" in this specification and claims is not intended to imply that color formation is a precipitation in the usual sense. The substance causing the color in the final product is usually a water-insoluble substance but is not necessarily produced in the presence of water.

15 The substance capable of donating sulfide ion at temperatures in excess of about 200° F. and stable in aqueous solution at temperatures below about 100° F. (hereinafter called "sulfide donor") is advantageously sodium thiosulfate. The sulfide donor is generally a sulfur-containing substance capable of dissolving in water in an amount to provide at least about 0.1% of sulfur available for reaction. Operable sulfide donors include ammonium thiosulfate, potassium thiosulfate, thiourea (thiocarbamide), and substituted thioureas in addition to sodium thiosulfate.

20 Thickening agents operable in the present invention include a colloidal suspension of boehmite-type aluminum oxide known in the trade as "Baymal," soluble starches such as arrowroot starch, hydroxy alkyl celluloses (e.g. hydroxyethyl cellulose), polyvinyl alcohol, polyacrylamide, methyl vinyl ether copolymer with maleic anhydride sold under the trade name "Gantrez AN," polyvinylpyrrolidone and an ethylene oxide polymer such as sold under the trade name "Polyox WSR Resin." Such thickening agents are employed in amounts of about 0.1 and up to about 20 or even 50 or more parts by weight of thickening agent per 100 parts by weight of water. Because of ionic effects on the viscosity of a colloidal suspension, it is impossible to specify with accuracy the exact amount of thickening agent needed to achieve the required viscosity without specifying the character and amount of each 25 ionic species present in impregnating composition of the present invention. It will be found, however, that an amount of thickening agent in the range of parts by weight, as specified hereinbefore, will usually suffice to achieve the required viscosity.

The use of a stabilizing agent in the coloring solutions of the present invention which contain sodium thiosulfate is highly advantageous and in some instances essential if one is to be assured that the coloring bath is to be stable for even short periods of time. It is possible for unstabilized solutions to exist for a measurable period of time without the appearance of precipitated sulfide. Such solutions can be used, for example, by being mixed in a spraying device immediately prior to spray application. In some instances where a bath life in excess of about 15 minutes or a half hour is not necessary, unstabilized baths may be used for dip, roller or other types of coating. In the usual case, however, it is highly advantageous to employ at least about 0.1% by weight of sodium or potassium bisulfite in the bath as a stabilizing agent. It is even more advantageous to employ at least about 0.3% of such stabilizing agent in the bath. Normally no more than about 1% of stabilizing agent is necessary but up to about 5% by weight or more can be used if desired. In the case of sodium thiosulfate solutions containing the cuprous ion as the sole coloring ion, the presence of at least about 0.3% by weight of stabilizing agent is a practical necessity since such solutions often can deteriorate by precipitation in very short spaces of time. Except for molybdenum solutions, all the sodium thiosulfate solutions of the present invention appear to be stable at the pH produced by the ingredients, which pH's are normally slightly acidic (i.e., a pH of 4 to 6). The pH of molybdenum-containing solutions must be adjusted to at least as high as about 7. Impregnating (coloring) compositions or solutions of the present invention containing thiourea appear to be shelf stable at least for several months without any stabilizing addition.

Optionally, but nevertheless highly advantageously, one can employ up to about 50% by weight or more (based on weight of solution but not included therein) of a flattening agent. A flattening agent for purposes of this specification and claims is a finely divided, essentially inert substance such as titanium dioxide (pigment grade), rouge (iron oxide), finely ground mica, finely divided chemically stabilized clay or the like. For dipping or spraying purposes, the use of a flattening agent in an amount within the aforesaid range and more particularly within about 5% to 20% by weight dispersed in the coloring solution is highly advantageous. The flattening agent enhances evenness of coverage of the metal to be colored and, in general, improves the workability of the coloring compositions.

As is obvious to one skilled in the art, the impregnating composition will contain addition ions balancing the color-producing ion in stoichiometrically equivalent amounts to permit electronic balance in the aqueous solution of the impregnating composition. These complementing ions necessarily are such that, together with the metal-bearing ion, they will produce a water soluble material stable in aqueous solution. Where mixtures of metallic species are employed, it is necessary to avoid mutually incompatible ions. For instance, one could not employ cobalt sulfate and lead acetate together in the same aqueous solution since metathesis dictates in this case the formation of lead sulfate an undesirable, substantially water-insoluble material. In like manner, salts, such as cobalt chloride and silver sulphate, are also mutually incompatible in an aqueous solution.

The base metal which is colored by means of the present invention is usually aluminum (including for purposes of this specification and claims anodizable alloys containing more than about 80% aluminum) but can be another anodizable metal such as titanium. In preparing aluminum for the coloring process of the present invention, it is usually necessary to anodize in such fashion as to produce a surface anodic film at least about 0.1 mil thick. For architectural purposes it is advantageous that the anodic film be at least about 0.5 mil thick, for example about 0.7 mil or thicker. Those skilled in the art will recognize that such anodic films may be produced in a number of different ways. In order to describe the invention with the utmost

particularity, however, details concerning satisfactory anodizing conditions in aqueous, acidic baths are set forth in Table I.

TABLE I

|                              | Broad aspect                      | Preferred aspect               |
|------------------------------|-----------------------------------|--------------------------------|
| Type of electrolyte          | H <sub>2</sub> SO <sub>4</sub>    | H <sub>2</sub> SO <sub>4</sub> |
| Concentration of electrolyte | 4 to 30% by weight                | 15% by weight                  |
| Anodic C.D.                  | 2 to 100 amps./ft. <sup>2</sup> * | 10 amps./ft. <sup>2</sup>      |
| Time                         | 0.5 to 90 minutes                 | 40 minutes                     |
| Temperature                  | 25 to 100° F                      | 72° F                          |

\* Amps./ft.<sup>2</sup>=amperes per square foot.

It is to be noted that while preferred conditions of anodizing have been set forth in Table I under the heading "Preferred Aspect," these preferred conditions are, in truth, designed to provide a satisfactory anodized coating about 0.7 mil thick on an aluminum alloy known to the art as grade 6063 containing nominally in percent by weight about 0.45 to 0.90% magnesium, about 0.2 to 0.6% silicon, not more than 0.35% iron, 0.1% each of copper, manganese, chromium, zinc and titanium in addition to aluminum. As those skilled in the art will recognize, each aluminum alloy will require subtle adjustments of the anodizing conditions within the broad range set forth in Table I to produce an equivalent coating. Since it may be possible to produce equivalent coatings in a non-electrolytic manner, the term "anodizing" is used in this specification and claims to include any and all means of forming a porous, adherent surface coating at least about 0.1 mil thick, which coating is substantially equivalent to those coatings produced under the broad conditions set forth in Table I.

Once the anodizing has been completed, the anodized object is rinsed and allowed to dry at about room temperature. The thickened solution of the coloring impregnant of the present invention is then applied to the anodized surface. While the thickened solution can be applied in any fashion which will produce an evenly distributed wet coating, it has been found to be advantageous to spray the thickened solution onto substantially horizontally oriented surfaces. It is possible and may at times be advantageous to arrange matters such that thickening of the solution occurs immediately prior to or simultaneously with the spraying. In this manner it is possible to employ thickening agents which, after a time, will become unstable in the presence of ionic solutions. After the freshly anodized surface has been sprayed with the thickened solution, it is immediately heated to a temperature of about 250° F. to about 1100° F. for about 2 to about 60 minutes. Generally it is advantageous to heat within the range of about 300° F. to about 600° F. with the greatest amount of control and flexibility being obtained when heating is conducted within the range of 350° F. to 450° F. It has been found satisfactory to heat to a temperature of about 400° F. for about 15 minutes. The heating can be accomplished by using an oven, by induction heating or by any other heating means known to the art, which heating means will not disturb the treated surface of the anodized metal. In further explanation of the heating operation, it is to be understood that when it is stated that a treated surface is heated to a temperature of about 400° F. for 15 minutes, this procedure is carried out when a wet, treated sheet metal object is introduced into an oven having an ambient temperature maintained within plus or minus 10° in Fahrenheit units of 400° F. It is recognized that attainment of the oven temperature by an object introduced therein is subject to a lag, especially when the surface of the object is wetted with an aqueous solution. Further, it is recognized that the mass of an object introduced into an oven is a determining factor as to the speed with which the object attains oven temperature. Accordingly, for purposes of this specification, temperatures and times are given with the understanding that sheet metal objects are being treated and that the oven or other heating means is of a sufficient capacity to heat a sheet metal object without losing temperature to any substantial degree. As

those skilled in the art will readily recognize, modifications of the time and/or temperature ranges may have to be made if conditions or situations other than those specifically described herein are encountered. After heating, anodized and colored aluminum is usually found to be sealed as shown by the ASTM Dye Test Designation B-136-63T—"Resistance of Anodically Coated Aluminum to Staining by Dyes." In some instances, such as when treating 1100 alloy, only partial sealing is attained.

For further corrosion protection the anodized and colored aluminum can be treated with polar aliphatic compounds, lacquers, waxes, boiling water, heated aqueous metal salt baths such as sodium dichromate, nickel acetate, etc. Treating with boiling water gives a velvety appearance to a black colored aluminum which at times may be desirable.

In carrying the present invention into practice, the concentration of the various reactants (color forming metal salt and precipitant) and control agents may vary widely. For example, the color forming salt may be used from a 1% concentration up to saturation, about 5-15% being usually advantageous. The sulfide donor can be used from a 1% concentration up to saturation, about 15 to 30% being usual. The solution stabilizing agent can be used from a 0.1% concentration up to about 3%, e.g. about 0.75 to about 1.25%. The flattening agent can be used from a 1% concentration up to 50% or more. About 2-8% of flattening agent is usually sufficient. The thickening agent concentration is governed by the ionic effects on the viscosity of a colloidal suspension. Thus, the thickening agent can sometimes be present in minute amounts or can be present up to concentrations that will form very viscous solutions. A particularly advantageous range for "Baymal" alumina is about 1 to 10%, e.g. 2-4%.

In carrying the present invention into practice, it is advantageous to employ as a blackening impregnant an aqueous composition made up with the following:

| Substance:                      | Amount in percent by weight |
|---------------------------------|-----------------------------|
| Cobalt chloride hexahydrate     | 4 to 15                     |
| Sodium thiosulfate pentahydrate | 12 to 30                    |
| Sodium bisulfite                | 0.5 to 1.25                 |
| Rouge ( $Fe_2O_3$ )             | 2 to 8                      |
| "Baymal"                        | 1 to 4                      |
| Water                           | Balance                     |

Blackening is accomplished by impregnating an anodized aluminum surface with the cobalt-containing ingredient and thereafter heating for about 15 minutes in an oven maintained at 400° F.

For the purpose of giving those skilled in the art a better appreciation of the advantages of the invention, the following specific examples are given:

#### EXAMPLE I

A sheet of aluminum alloy designated as grade 6063 and containing in addition to aluminum about .45-.90% of magnesium and about .20-.60% of silicon was anodized in a 15% sulfuric acid-water bath at 72° F. for about 60 minutes to produce an anodic film about 0.1 mil thick. The anodized alloy was then dried in air at room temperature (i.e., about 72° F.) The anodized alloy was then sprayed with an impregnating composition prepared as follows:

##### Master solution

|                          | Gm. |
|--------------------------|-----|
| $Na_2S_2O_3 \cdot 5H_2O$ | 250 |
| $NaHSO_3$                | 10  |
| $CoCl_2 \cdot 6H_2O$     | 100 |

To 700 ml. deionized water add the above ingredients and when dissolved dilute to 1 liter with water.

##### Solution for spraying

In a high speed blender, blend

300 ml. of master solution

20 gm. rouge ( $Fe_2O_3$ )

100 ml. 10% "Baymal" in water

The impregnated anodized sheet was then heated in an oven at 400° F. for about 15 minutes. After washing off excess material the anodized surface was found to be colored jet black. It is to be observed that the procedure followed in this and subsequent examples is that procedure illustrated in schematic form on the drawing. Referring now thereto, it is to be noted that the two-step process of the invention involving coating with impregnant (or more broadly speaking, impregnating), and heating is preceded by the conventional anodizing operations and followed by any necessary cleaning and sealing operations.

#### EXAMPLE II

Aluminum alloy 6063 is anodized as in Example I. A sample of the anodized alloy is impregnated by immersing in coloring solution and withdrawn at the rate of about 3" per minute. Solution composition is as follows:

|                         | Gm. |
|-------------------------|-----|
| $CoCl_2 \cdot 6H_2O$    | 100 |
| $(NH_2)_2CS$ (thiourea) | 100 |

Arrowroot starch 3% to 1 liter.

Dissolve the above salts in approximately 700 ml. of 3% aqueous solution of arrowroot starch. When dissolved dilute to 1 liter with the starch.

Aluminum sheet after impregnation heated as in Example I.

#### EXAMPLE III

A buffed sheet of aluminum alloy designated as grade 305457 and containing in addition to aluminum about .80-1.20% magnesium, about .15-.45% manganese and about .20% copper, .10% iron and .08% silicon was anodized in a 15%  $H_2SO_4$  water bath at 72° F. for about 40 minutes to produce an anodic film about 0.5 mil thick. The anodized alloy divided into two parts was then dried in air at room temperature, treated as in Examples I and II and heated to 400° F. for 15 minutes. Excess salts were removed by washing with water. A bright jet black color was obtained.

#### EXAMPLE IV

Aluminum alloy 6063, anodized as in Example I, was sprayed with an impregnating composition prepared as follows:

##### Master solution

|                          | Grams |
|--------------------------|-------|
| $Na_2S_2O_3 \cdot 5H_2O$ | 250   |
| $NaHSO_3$                | 10    |
| $CuCl$                   | 50    |

Dissolve the  $Na_2S_2O_3 \cdot 5H_2O$  and  $NaHSO_3$  in approximately 700 ml. of  $H_2O$ . When dissolved add the  $CuCl$  and when dissolved dilute to 1 liter.

##### Solution for spraying

In a high speed blender, blend

300 ml. master solution

20 gm. rouge ( $Fe_2O_3$ )

200 ml. 10% "Baymal"

After heating and cleaning, as described in Example I, a dark green color was obtained in the anodized layer.

#### EXAMPLE V

Aluminum alloy 6063, anodized as in Example I, was sprayed with an impregnating composition prepared as follows:

##### Master solution

|                                 | Grams |
|---------------------------------|-------|
| $Na_2S_2O_3 \cdot 5H_2O$        | 250   |
| $NaHSO_3$                       | 10    |
| $CdCl_2 \cdot 2\frac{1}{2}H_2O$ | 100   |

Dissolve the above salts in approximately 700 ml. deionized  $H_2O$ . When dissolved dilute to 1 liter with  $H_2O$ .

## Solution for spraying

In a high speed blender, blend

400 ml. master solution  
 20 gm. rouge ( $Fe_2O_3$ )  
 150 ml. 10% "Baymal"

After heating and cleaning, as described in Example I, a bright canary yellow color was obtained in the anodized layer.

## EXAMPLE VI

Aluminum alloy 6063 is anodized as in Example I. The anodized alloy was then sprayed with an impregnating composition prepared as follows:

## Master solution

|                          | Grams |
|--------------------------|-------|
| $Na_2S_2O_3 \cdot 5H_2O$ | 250   |
| $NaHSO_3$                | 10    |
| CuCl                     | 25    |
| $(NH_4)_6Mo_7O_24$       | 50    |

Dissolve the first two salts in approximately 700 ml. deionized water. When dissolved, dissolve the third and then the fourth salt. When dissolved immediately, adjust pH to 7.0 with  $NH_4OH$  and dilute to 1 liter with  $H_2O$ .

## Solution for spraying

In a high speed blender, blend

350 ml. master solution  
 20 gm. rouge ( $Fe_2O_3$ )  
 100 ml. 10% "Baymal"

After heating and cleaning, as described in Example I, a red-brown color was obtained in the anodized layer.

Additional examples of anodized alloys treated in accordance with the present invention are set forth in the following table together with the colors produced.

| Alloy            | Solution                | Heating temp.,<br>°F. | Time<br>(min.) | Color produced |
|------------------|-------------------------|-----------------------|----------------|----------------|
| Titanium.....    | Solution of Example I.  | 400                   | 15             | Black.         |
| Al Alloy 1100... | Solution of Example IV. | 400                   | 15             | Dark Green.    |
| Al Alloy 7075... | Solution of Example I.  | 400                   | 15             | Black.         |
| Al Alloy 7075... | Solution of Example V.  | 400                   | 15             | Yellow.        |

Colored anodized metal, e.g. aluminum, produced in accordance with the present invention, is particularly adapted for architectural uses on the exterior of buildings and in any other locations where exposure to sunlight exists. The colors produced are resistant to fading in sunlight and are resistant to the detrimental action many substances carried in normal urban atmospheres. Many other uses can be contemplated for aluminum colored in accordance with the present invention. For example, attractive effects can be produced by combining the coloring procedure of the present invention with other metal treatments such as pre-anodizing, texturing, partial masking of surfaces during impregnation of the coloring solutions of the present invention and the like, which effects can be employed wherever decorated metal is required. Above and beyond mere decoration, the process of the present invention can be employed to provide surfaces which absorb or radiate moderate amounts of heat and thus provide utilitarian as well as aesthetic effects.

Although the present invention has been described in conjunction with preferred embodiments, it is to be understood that modifications and variations may be resorted to without departing from the spirit and scope of the invention, as those skilled in the art will readily understand.

Such modifications and variations are considered to be within the purview and scope of the invention and appended claims.

I claim:

5. A process for producing a color on anodized metal comprising impregnating a porous anodized layer on said metal with a stable, aqueous solution containing both a precipitant ion donor and an ion, said solution being unstable at an elevated temperature of a metal capable of forming a colored precipitate with said precipitant ion and subsequently heating the thus impregnated anodized layer at a temperature effective to induce formation of said colored precipitate.
10. 2. A process as in claim 1 wherein the precipitant ion is sulfide ion.
15. 3. A process as in claim 2 wherein the sulfide donor is a substance selected from the group consisting of sodium thiosulfate, potassium thiosulfate, ammonium thiosulfate, thiourea and substituted thioureas.
20. 4. A process as in claim 2 wherein the sulfide donor is sodium thiosulfate and the metal capable of forming a colored sulfide is selected from the iron group metals.
25. 5. A process for producing a color on anodized metal comprising impregnating a porous anodized layer on said metal with a stable aqueous solution containing a metalliferous ion from the group of cobalt, copper, antimony, nickel, molybdenum, iron, and bismuth ions, sodium thiosulfate and at least about 0.1% by weight of sodium bisulfite and, thereafter, heating the thus impregnated porous anodized layer at a temperature in excess of about 250° F. for at least about one minute.
30. 6. A process as in claim 5 wherein the sodium bisulfite is present in at least about 0.3% by weight.
35. 7. A process as in claim 5 wherein the metalliferous ion is an ion of the iron group metals.
8. A process as in claim 5 wherein the heating is conducted for about 15 minutes at a temperature of about 400° F.
40. 9. A process as in claim 5 wherein the stable aqueous solution has a flattening agent dispersed therethrough.
45. 10. As a composition of matter an aqueous solution containing dissolved therein at least one metal bearing ion bearing a metal from the group consisting of cobalt, copper, antimony, nickel, molybdenum, iron, and bismuth, a sulfide donor from the group consisting of sodium thiosulfate, potassium thiosulfate, ammonium thiosulfate, thiourea and substituted thioureas, a thickening agent and, at least when copper is the sole metal bearing ion and when a thiosulfate is the sulfide donor, an effective amount of sodium bisulfite up to about 5% by weight to stabilize said solution.
50. 11. A composition of matter as in claim 10 wherein the solution also has dispersed therethrough up to about 50% by weight of a flattening agent.
55. 12. A composition of matter as in claim 10 wherein the sulfide donor is sodium thiosulfate and the metal is an iron group metal.
60. **References Cited**
- UNITED STATES PATENTS
- 2,018,388 10/1935 Tosterod ----- 204—35  
 3,152,970 10/1964 Jensen ----- 204—35
65. JOHN H. MACK, Primary Examiner.  
 R. L. ANDREWS, Assistant Examiner.
70. U.S. Cl. X.R.  
 148—6.24, 6.27; 204—35